

# United States Patent [19]

Goodman, Jr. et al.

[11] 3,871,822

[45] Mar. 18, 1975

[54] **TREATMENT OF CELLULOSIC TEXTILE FABRICS WITH METHYLOLATED ALKOXYALKYL CARBAMATES**

[75] Inventors: **Henry G. Goodman, Jr.**, White Plains; **Carol A. Dupraz**, Flushing (Corona); **George H. Lourigan**, New City, all of N.Y.

[73] Assignee: **Union Carbide Corporation**, New York, N.Y.

[22] Filed: **Feb. 16, 1966**

[21] Appl. No.: **527,772**

[52] U.S. Cl. .... **8/187**, 8/115.7, 260/482 C

[51] Int. Cl. .... **D06m 13/40**, D06m 15/54

[58] Field of Search. .... 8/116.3, 187; 260/482 C

[56] **References Cited**

UNITED STATES PATENTS

2,774,746 12/1956 Shelly et al. .... 8/116.3 X

3,391,181 7/1968 Scheuerl ..... 260/482  
3,524,876 8/1970 Gregson ..... 8/116.3 X

Primary Examiner—George F. Lesmes

Assistant Examiner—J. Cannon

Attorney, Agent, or Firm—Francis M. Fazio

[57]

## ABSTRACT

The invention relates to treatment of cellulosic textile fabrics with methyolated alkoxyalkyl carbamate finishing agents to impart improved wrinkle and shrink resistance thereto. The novel finishing agents are prepared by reaction of formaldehyde with an alkoxyalkyl carbamate such as methoxyethyl carbamate. Methyolated alkyl carbamates and methyolated hydroxyalkyl carbamates have been employed for this same purpose in the past, but the methyolated alkoxyalkyl carbamates of the present invention provide treated fabrics which exhibit superior properties.

4 Claims, No Drawings

**TREATMENT OF CELLULOSIC TEXTILE  
FABRICS WITH METHYLOLATED  
ALKOXYALKYL CARBAMATES**

This invention relates to the preparation of textile fabrics having improved wrinkle and shrink resistance and other improved properties. More specifically, this invention relates to a process for treating cellulosic textile fabrics with methyolated alkoxyalkyl carbamates and to the treated fabrics produced thereby.

One of the important recent developments in the finishing of cellulosic textile fabrics has been the introduction of finishing agents prepared by reacting aliphatic monocarbamates with formaldehyde. These products have been found to be very effective in imparting wrinkle resistance and wash-wear properties to the fabric, while displaying the important advantages, as compared with conventional nitrogenous finishing agents, of enhanced resistance to chlorine damage and durability under conditions promoting acid hydrolysis. Heretofore, finishing agents of this type have been prepared from alkyl carbamates, such as methyl, ethyl, propyl or butyl carbamate, or from hydroxyalkyl carbamates, such as hydroxyethyl carbamate, and have been observed from certain deficiencies, for example, with regard to abrasion resistance, tear strength and fabric hand, which have hindered their optimum commercial development. Moreover, these finishing agents, though greatly superior to conventional nitrogenous finishing agents such as dimethylol ethyleneurea or methylated methyolmelamine with respect to resistance to chlorine damage and durability to acid hydrolysis, are, in certain instances, still somewhat deficient in this regard. It is toward the objectives of overcoming these deficiencies and of providing treated textile fabrics of improved properties that the present invention is directed.

This invention is based on the discovery that finishing agents for treating cellulosic textile fabrics which are prepared by reaction of formaldehyde with an alkoxyalkyl carbamate, as hereinafter define, permit the preparation of fabrics with superior properties as compared to the finishes derived from alkyl or hydroxyalkyl carbamates in accordance with the teachings of the prior art. It was unexpected and surprising to find that the methyolated alkoxyalkyl carbamates described herein are superior finishing agents to both the methyolated alkyl carbamates and methyolated hydroxylalkyl carbamates. While applicants do not intend to be bound by any theoretical considerations, it is believed that this superior performance is predicated, to a degree, on the superior lubricating properties of the methyolated alkoxyalkyl carbamates, since fiber lubricity is an important factor in determining many fabric properties.

The alkoxyalkyl carbamates employed in preparing the textile treating agents of this invention are compounds of the general formula:



wherein R is an alkyl group of 1 to 8 carbon atoms and preferably of 1 to 4 carbon atoms, R' is an alkylene radical of 2 to 3 carbon atoms, and n is an integer having

a value of from 1 to 10, and preferably of from 1 to 3. They may be prepared by any of several methods known to the art. A particularly convenient method of preparation involves the reaction of urea with a glycol ether of the formula:



where R, R' and n are as defined above, to form the alkoxyalkyl carbamate and liberate ammonia. Illustrative of the glycol ethers within the scope of this definition are the methyl, ethyl, butyl, isobutyl, hexyl and 2-ethylhexyl ethers of ethylene glycol, propylene glycol, diethylene glycol, dipropylene glycol, triethylene glycol, tripropylene glycol, polyethylene glycol, polypropylene glycol, and mixed polyethylene-polypropylene glycol.

The alkoxyalkyl carbamates described above are reacted with formaldehyde to produce the methyolated alkoxyalkyl carbamates having utility as textile finishing agents in accordance with this invention. The exact structure of the reaction product of formaldehyde with the alkoxyalkyl carbamate has not been established, but it is believed that a mixture of monomethylol and dimethylol derivatives results, viz., a mixture of an N-methylol alkoxyalkyl carbamate of the formula:



and an N,N-dimethylol alkoxyalkyl carbamate of the formula:



where R, R' and n are as defined hereinabove. In addition to the combined formaldehyde in the reaction product represented by the methyl radicals, some of the formaldehyde is believed to be present as free formaldehyde and some as combined formaldehyde which is present in a form which has not yet been established.

Although the conditions under which the methylation reaction is effected significantly affect the performance characteristics of the reaction product, the reaction conditions are not narrowly critical. A suitable procedure is to dissolve the alkoxyalkyl carbamate in water, add the formaldehyde to the aqueous solution, adjust the pH to the desired level, and then heat the mixture for the period necessary to effect methylation. Upon cooling, neutralization, dilution with water, and filtration, the product is recovered as a clear, colorless solution of the methyolated alkoxyalkyl carbamate.

The reaction of formaldehyde and the alkoxyalkyl carbamate may be effected at temperatures from about 20°C., preferably about 50°C., to the reflux temperature of the reaction mixture, i.e., slightly above 100°C. Reaction times of from about 10 minutes to about 24 hours, and preferably from about 1 to 5 hours, may be employed. The initial pH of the reaction mixture

should be from about 4 to about 10, and preferably from about 8 to about 10.

The most important factor in determining the performance of the finishing agents is the ratio of formaldehyde to alkoxyalkyl carbamate employed. The reaction products of particular utility for the purposes of this invention are those prepared by reacting the formaldehyde with the alkoxyalkyl carbamate in a molar ratio of from about 1.5 to about 3 moles of formaldehyde per mole of alkoxyalkyl carbamate, and preferably in a molar ratio of from about 2 to about 2.5.

Textile fabrics which are amenable to treatment with the finishing agents of this invention are the cellulosic textile fabrics. The term "cellulosic textile fabric," as used throughout the specification and in the appended claims, is intended to include fabrics, whether woven or knitted, and garments or other articles made from such fabrics, and is also intended to include both cellulose fabrics, including regenerated cellulose, and cellulose-containing fabrics. The cellulosic textile fabrics comprehended thus include cotton fabrics, linen fabrics, rayon fabrics, fabrics consisting of blends of cotton, linen or rayon fibers, and fabrics consisting of blends of cellulose fibers and non-cellulosic fibers.

The finish may be applied to the cellulosic textile fabric in any suitable manner known to the art, for example, by dipping or padding. Ordinarily, the finishing agent, which term is employed herein to mean the reaction product of formaldehyde and the alkoxyalkyl carbamate, is applied to the fabric from aqueous solution. Such aqueous treating solution may, if desired, contain, in addition to the finishing agent, other materials employed in textile finishing such as plasticizers, softening agents, hand builders, and the like.

The amount of finishing agent to be applied to the fabric varies widely depending upon the type of fabric and its intended application, and, accordingly, the present invention comprehends the use of any effective amount. Amounts of from about 1 to about 30 per cent by weight of the finishing agent, based on the weight of the textile fabric, are ordinarily employed, i.e., an add-on of about 1 to about 30 per cent. It is preferred to employ an amount of at least about 4 per cent. In any particular finishing operation the add-on will depend upon the concentration of the finishing agent in the treating solution and the weight of solution which the textile fabric will retain, i.e., the wet pick-up. A wet pick-up of from about 50 to about 120 per cent may be readily effected by conventional techniques, while the treating solution applied to the textile fabric in practicing this invention may contain from as little as about 2 per cent, or less, to as much as about 25 per cent, or more, of the finishing agent. Accordingly, no difficulty is encountered in achieving the desired add-on.

The methyloolated alkoxyalkyl carbamates of this invention, like the nitrogenous textile finishing agents of the prior art, require curing following application to the textile fabric to promote reaction with the fibers of the fabric and thereby impart the desired properties, such as wrinkle resistance and wash-wear characteristics. Suitable catalysts for the curing reaction are metal salts of strong mineral acids, particularly zinc fluoborate and the hydrates of magnesium chloride and zinc nitrate. The catalyst is ordinarily added to the aqueous treating solution and should be employed in a concentration sufficient to give a retention of catalyst of about 0.5 to about 5 weight per cent, based on the weight of the fab-

ric. Larger amounts of catalyst, within the range specified, are preferably employed at the higher add-on levels of the finishing agent. The optimum amount of catalyst varies depending on the particular catalyst employed. For example, with magnesium chloride it is preferred to utilize a ratio of catalyst to finishing agent by weight, as retained on the fabric, of from about 0.2 to about 0.6, while with zinc nitrate or zinc fluoborate the preferred ratio is from about 0.05 to about 0.2.

Following application of the aqueous treating solution, the fabric is subjected to heating to remove the water and then curing is effected by the application of further heat. It is preferred to dry the fabric at temperatures lower than those employed in the curing. Thus, drying is usually carried out at temperatures of up to about 150°C., while temperatures from 150°C. to about 200°C. are ordinarily employed in the curing step. The time required to effect the curing will vary from as little as about 1 minute, or less, to as much as about 5 minutes, or more. Normal curing, i.e., curing immediately after drying, or deferred curing, i.e., after the fabric has been made into a garment, may be employed as desired.

Resistance to chlorine damage caused by hypochlorite bleaching and durability to conditions promoting acid hydrolysis, such as acid scouring, are important considerations in the art of finishing cellulosic textile fabrics. Textile fabrics treated by the method of this invention are, in many instances, possessed of superior resistance to chlorine damage and/or enhanced durability to acid hydrolysis as compared with fabrics treated with the methyloolated alkyl and hydroxyalkyl carbamates of the prior art. In particular, it has been found that the methyloolated alkoxyalkyl carbamates are, in general, equivalent in resistance to chlorine damage to the methyloolated alkyl carbamates, but superior in durability to acid hydrolysis. On the other hand, the methyloolated alkoxyalkyl carbamates have been found to be, in general, equivalent in durability to acid hydrolysis to the methyloolated hydroxyalkyl carbamates, but superior in resistance to chlorine damage particularly in that they exhibit excellent resistance to chlorine damage even when the fabric treating and curing conditions are varied widely whereas the methyloolated hydroxyalkyl carbamates exhibit undesired criticality as regards the fabric treating and curing conditions necessary. These are important and unexpected differences which, in part, serve to distinguish the present invention from the prior art.

In addition to their excellent resistance to acid hydrolysis, and consequent durability to laundering, and their ability to provide a fabric which will not be harmed by hypochlorite bleaching, the methyloolated alkoxyalkyl carbamate finishing agents described herein provide improved abrasion resistance and, in certain instances, a more desirable hand, as compared with the methyloolated alkyl and hydroxyalkyl carbamates. Moreover, they are more efficient on a molar basis and equally as efficient on a weight basis as the prior art finishing agents.

Evaluation of textile fabrics treated by the process of this invention was in accordance with test procedures of the American Society for Testing Materials (ASTM) or the American Association of Textile Chemists and Colorists (AATCC), or by procedures that are fully described herein. The following tests were conducted:

Wash-Wear Rating — determined by AATCC Tentative Test Method 88A-1964T. The rating, which is indicative of the smoothness of appearance of the fabric, ranges from 1 to 5 with intermediate ratings indicated by + and - symbols.

Crease Recovery — measured by AATCC Tentative Test Method 66-1959T.

Tensile Strength — measured by ASTM Method D39-49 (Grab Test)

Tear Strength — measured by ASTM Method D1424-56 (Elmendorf)

Abrasion Resistance — measured by ASTM Method D1175-51T-B.

Damage Due to Retained Chlorine — measured by AATCC Standard Method 92-1962.

Durability to Acid Hydrolysis — samples of treated fabric were hydrolyzed for 30 minutes at 60-65°C. in Clark and Lubs buffer solutions at controlled pH, then washed in cold water, ironed dry, conditioned, and tested for dry crease recovery.

The invention is further illustrated by the following specific examples of its practice

#### EXAMPLE I

To a reaction flask there were charged 119 grams of methoxyethyl carbamate (prepared by reacting urea with ethylene glycol monomethyl ether), 66 grams of p-formaldehyde, and 120 grams of water (a molar ratio of formaldehyde to methoxyethyl carbamate of 2.2 to 1). The pH of the slurry was adjusted to 10 by addition of 10% NaOH and then it was refluxed for 2 hours to form the methylolated methoxyethyl carbamate, whereupon it was neutralized, diluted with water to 50% active material, and filtered.

Samples of desized, scoured, bleached and mercerized white cotton printcloth having a thread count of 80 x 80 were padded with a treating bath containing the methylolated methoxyethyl carbamate using a Butterworth Laboratory Padder. In each instance, the treating bath was composed of methylolated methoxyethyl carbamate, MgCl<sub>2</sub> · 6H<sub>2</sub>O, Fabritone PE (a commercial softner composed of emulsified polyethylene was of 30% solids content) and TERGITOL TMN

(trade-mark for a nonionic surfactant characterized as a trimethyl nonyl ether of polyethylene glycol) with the balance being water. After treatment, the wet fabric was placed on a pin tenter frame, dried at 150°C. for 1.5 minutes, and cured at 175°C. for 1.25 minutes.

15 For comparison purposes, identical samples of the cotton print-cloth were treated in the same manner as described above, but employing methylolated ethyl carbamate in place of the methylolated methoxyethyl carbamate. The methylolated ethyl carbamate was prepared under the same reaction conditions at a formaldehyde to ethyl carbamate mole ratio of 2.2 to 1 (the reaction mixture consisting of 89 grams of ethyl carbamate, 66 grams of p-formaldehyde and 90 grams of water) and the treated fabric samples were dried and

20 cured under identical conditions to those described above in connection with the methylolated methoxyethyl carbamate. The treating bath compositions and the add-on levels, which were the same in each particular run for both the methylolated methoxyethyl carbamate and the methylolated ethyl carbamate, are summarized in Table I below: while the properties of the treated fabric are summarized in Table II, fabric samples treated with methylolated ethyl carbamate being designated by the letter A and those treated with

25 methylolated methoxyethyl carbamate by the letter B.

TABLE I

| Run No. | Treating Bath (% by weight) |                                       |              |              | Add-On (% on weight of fabric) |                                       |              |  |
|---------|-----------------------------|---------------------------------------|--------------|--------------|--------------------------------|---------------------------------------|--------------|--|
|         | Finishing Agent             | MgCl <sub>2</sub> · 6H <sub>2</sub> O | Fabritone PE | TERGITOL TMN | Finishing Agent                | MgCl <sub>2</sub> · 6H <sub>2</sub> O | Fabritone PE |  |
| 1       | 5.0                         | 1.0                                   | 1.8          | 0.1          | 2                              | 0.8                                   | 0.4          |  |
| 2       | 7.5                         | 1.5                                   | 1.8          | 0.1          | 3                              | 1.2                                   | 0.4          |  |
| 3       | 10.0                        | 2.0                                   | 1.8          | 0.1          | 4                              | 1.6                                   | 0.4          |  |
| 4       | 12.5                        | 2.5                                   | 1.8          | 0.1          | 5                              | 2.0                                   | 0.4          |  |
| 5       | 15.0                        | 3.0                                   | 1.8          | 0.1          | 6                              | 2.4                                   | 0.4          |  |
| 6       | 17.5                        | 3.5                                   | 1.8          | 0.1          | 7                              | 2.8                                   | 0.4          |  |
| 7       | 20.0                        | 4.0                                   | 1.8          | 0.1          | 8                              | 3.2                                   | 0.4          |  |

TABLE II

| Fabric Sample | Dry Crease Recovery Warp + Filling (degrees) | Tear Strength Warp + Filling (grams) | Tensile Strength Filling (lbs.) | Wash-Wear Rating |          | Abrasion Resistance (cycles to break) | Dry Crease Recovery After Hydrolysis at pH of 2 |
|---------------|----------------------------------------------|--------------------------------------|---------------------------------|------------------|----------|---------------------------------------|-------------------------------------------------|
|               |                                              |                                      |                                 | Tumble Dry       | Spin Dry |                                       |                                                 |
| 1-A           | 233                                          | 1270                                 | 19                              | 2+               | 2        | 691                                   | 204                                             |
| 1-B           | 232                                          | 1300                                 | 21                              | 2                | 2        | 894                                   | 214                                             |
| 2-A           | 268                                          | 1140                                 | 20                              | 3+               | 3        | 388                                   | 217                                             |
| 2-B           | 256                                          | 1120                                 | 23                              | 3                | 2        | 466                                   | 223                                             |
| 3-A           | 278                                          | 970                                  | 18                              | 4-               | 3+       | 313                                   | 237                                             |
| 3-B           | 277                                          | 1070                                 | 20                              | 4-               | 4-       | 400                                   | 243                                             |
| 4-A           | 291                                          | 910                                  | 19                              | 4+               | 4        | 207                                   | 243                                             |
| 4-B           | 287                                          | 960                                  | 17                              | 4+               | 4        | 281                                   | 258                                             |
| 5-A           | 285                                          | 870                                  | 19                              | 4+               | 4        | 170                                   | 246                                             |
| 5-B           | 288                                          | 930                                  | 19                              | 5-               | 3+       | 206                                   | 259                                             |
| 6-A           | 290                                          | 770                                  | 18                              | 5-               | 4        | 163                                   | 265                                             |
| 6-B           | 297                                          | 900                                  | 17                              | 5-               | 4+       | 174                                   | 261                                             |
| 7-A           | 297                                          | 750                                  | 17                              | 5-               | 4+       | 116                                   | 261                                             |
| 7-B           | 289                                          | 850                                  | 19                              | 5-               | 4+       | 161                                   | 274                                             |

As evidenced by the data in Tables I and II, the methylolated methoxyethyl carbamate finish of this invention, employed with fabric samples identified by the letter B, gives improved tear strength, abrasion resistance and durability to acid hydrolysis as compared with the methylolated ethyl carbamate of the prior art, employed with fabric samples identified by the letter A, while giving at least equal performance with regard to other fabric properties. Moreover, it was found that the methylolated methoxyethyl carbamate provides a treated fabric with a more pleasing hand than the fabric treated with methylolated ethyl carbamate.

#### EXAMPLE 2

Several methylolated alkoxyalkyl carbamates were prepared and evaluated as finishing agents for cotton

prepared by reaction of equimolar quantities of ethylene carbonate and ammonium hydroxide in aqueous solution at 0°C. to 10°C. for 2 hours, in a ratio of 2 moles of p-formaldehyde per mole of hydroxyethyl carbamate.

The carbamate finishing agents were applied to samples of desized, scoured, bleached and mercerized white cotton printcloth having a thread count of 80 × 80 at several levels of finish and catalyst add-on using a Butterworth Laboratory Padder. In each case, the catalyst employed was  $MgCl_2 \cdot 6H_2O$  and the treating bath contained 0.1 per cent by weight TERGITOL TMN. After treatment, the wet fabric was placed on a pin tenter frame, dried at 150°C. for 1.5 minutes, and cured at 175°C. for 1.25 minutes. The add-on levels and the properties of the treated fabric are summarized in Table III below.

Table III

| Finishing Agent                        | Add-On<br>(% on wt. of fabric) | Finishing Agent<br>$MgCl_2 \cdot 6H_2O$ | Dry Crease Recovery<br>Warp+Filling<br>(degrees) | Tear Strength<br>Warp+Filling<br>(grams) | Tensile Strength<br>Filling<br>(lbs) | Wash-Wear Rating<br>Tumble Dry<br>Spin Dry | Loss in<br>Tensile Strength<br>Due to<br>Retained Chlorine(%) |
|----------------------------------------|--------------------------------|-----------------------------------------|--------------------------------------------------|------------------------------------------|--------------------------------------|--------------------------------------------|---------------------------------------------------------------|
| Methylolated hydroxyethyl carbamate    | 4                              | 3                                       | 251                                              | 790                                      | 23                                   | 4 2+                                       | N.D. <sup>(1)</sup>                                           |
|                                        | 8                              | 1                                       | 256                                              | 900                                      | 28                                   | 3+ 2+                                      | N.D.                                                          |
|                                        | 8                              | 2                                       | 264                                              | 860                                      | 28                                   | 4 3                                        | N.D.                                                          |
|                                        | 8                              | 3                                       | 269                                              | 680                                      | 19                                   | 4 4-                                       | 74                                                            |
|                                        | 8                              | 4                                       | 276                                              | 810                                      | 25                                   | 4 4                                        | N.D.                                                          |
|                                        | 12                             | 3                                       | 260                                              | 690                                      | 22                                   | 5- 5-                                      | N.D.                                                          |
| Methylolated methoxyethyl carbamate    | 4                              | 3                                       | 255                                              | 660                                      | 24                                   | 4 2                                        | 10.5                                                          |
|                                        | 8                              | 1                                       | 237                                              | 850                                      | 24                                   | 4- 3+                                      | N.D.                                                          |
|                                        | 8                              | 2                                       | 266                                              | 710                                      | 24                                   | 4 3+                                       | N.D.                                                          |
|                                        | 8                              | 3                                       | 263                                              | 640                                      | 24                                   | 5- 4                                       | 13                                                            |
|                                        | 8                              | 4                                       | 273                                              | 550                                      | 23                                   | N.D. 4                                     | N.D.                                                          |
|                                        | 12                             | 3                                       | 267                                              | 660                                      | 21                                   | 5- 4                                       | 0                                                             |
| Methylolated ethoxyethyl carbamate     | 4                              | 3                                       | 247                                              | 610                                      | 18                                   | 4 3+                                       | N.D.                                                          |
|                                        | 8                              | 1                                       | 252                                              | 660                                      | 24                                   | 4- 3+                                      | N.D.                                                          |
|                                        | 8                              | 2                                       | 253                                              | 590                                      | 21                                   | 4 3                                        | N.D.                                                          |
|                                        | 8                              | 3                                       | 270                                              | 570                                      | 20                                   | N.D. N.D.                                  | 10                                                            |
|                                        | 8                              | 4                                       | 263                                              | 580                                      | 22                                   | 5- 4                                       | N.D.                                                          |
|                                        | 12                             | 3                                       | 272                                              | 580                                      | 23                                   | 5- 4                                       | N.D.                                                          |
| Methylolated butoxyethyl carbamate     | 4                              | 3                                       | 235                                              | 620                                      | 19                                   | 4- 2                                       | N.D.                                                          |
|                                        | 8                              | 1                                       | 229                                              | 720                                      | 29                                   | 3- 2-                                      | N.D.                                                          |
|                                        | 8                              | 2                                       | 237                                              | 660                                      | 26                                   | 4- 4-                                      | N.D.                                                          |
|                                        | 8                              | 3                                       | 256                                              | 600                                      | 20                                   | 4 3                                        | 0                                                             |
|                                        | 8                              | 4                                       | 263                                              | 560                                      | 22                                   | 4 4-                                       | N.D.                                                          |
|                                        | 12                             | 3                                       | 246                                              | 640                                      | 22                                   | 4 4                                        | N.D.                                                          |
| Methylolated iso-butoxyethyl carbamate | 4                              | 3                                       | 247                                              | 600                                      | 22                                   | 4- 3-                                      | N.D.                                                          |
|                                        | 8                              | 1                                       | 207                                              | 770                                      | 30                                   | 2- 1                                       | N.D.                                                          |
|                                        | 8                              | 2                                       | 226                                              | 640                                      | 26                                   | 3+ 2+                                      | N.D.                                                          |
|                                        | 8                              | 3                                       | 259                                              | 620                                      | 21                                   | 4 4-                                       | 0                                                             |
|                                        | 8                              | 4                                       | 258                                              | 580                                      | 26                                   | 5- 4-                                      | N.D.                                                          |
|                                        | 12                             | 3                                       | 247                                              | 640                                      | 22                                   | 4 2+                                       | N.D.                                                          |

<sup>(1)</sup>N.D. = not determined.

fabrics and methylolated hydroxyethyl carbamate was prepared and similarly evaluated for comparison purposes. The methylolated alkoxyalkyl carbamates were prepared by dissolving p-formaldehyde in an aqueous solution of the corresponding alkoxyalkyl carbamate (prepared by reaction of urea with the appropriate glycol ether in the presence of zinc acetate catalyst) in an amount of 2 moles of p-formaldehyde per mole of alkoxyalkyl carbamate, heating to about 80°C. to dissolve the p-formaldehyde, and then permitting the mixture to stand at room temperature for several hours. The methylolated hydroxyethyl carbamate was prepared by reacting p-formaldehyde with hydroxyethyl carbamate,

As evidenced by the data in Table III, the loss in strength of the fabric due to chlorine damage is very much less with the methylolated alkoxyalkyl carbamates of this invention as compared with the methylolated hydroxyethyl carbamate of the prior art. For example, at an add-on of 8% of finishing agent and 3% of catalyst, the strength loss due to retained chlorine was 74% with the methylolated hydroxyethyl carbamate as compared with a maximum of 13% for the four methylolated alkoxyalkyl carbamates evaluated. Moreover, the data indicate that the methylolated alkoxyalkyl carbamates provide, in general, at least comparable performance to the methylolated hydroxyethyl carbamate

as regards crease recovery, wash-wear characteristics, and fabric strength.

### EXAMPLE 3

This example demonstrates the effect of methylolation conditions on the performance of methylolated

tions under which the methylolation of the methoxyethyl carbamate was carried out and the properties of the fabric samples treated with the finishing agents produced under the differing conditions are summarized in Tables IV, V and VI for test series one, two, and three respectively.

TABLE IV

| Molar Ratio of Formaldehyde to Carbamate | Initial pH | Reaction time (hrs.) | Reaction Temperature (°C.) | Dry Crease Recovery Warp+Filling (degrees) | Tear Strength Warp+Filling (grams) | Tensile Strength, Filling (lbs.) | Loss in Tensile Strength Due to Retained Chlorine (%) |
|------------------------------------------|------------|----------------------|----------------------------|--------------------------------------------|------------------------------------|----------------------------------|-------------------------------------------------------|
| 1:1                                      | 10         | 2                    | 103                        | 199                                        | 1260                               | 28                               | N.D. <sup>(1)</sup>                                   |
| 1.5:1                                    | 10         | 2                    | 103                        | 237                                        | 1130                               | 23                               | N.D.                                                  |
| 2:1                                      | 10         | 2                    | 103                        | 257                                        | 1060                               | 22                               | N.D.                                                  |
| 2.5:1                                    | 10         | 2                    | 103                        | 268                                        | 1010                               | 22                               | 9                                                     |
| 3:1                                      | 10         | 2                    | 103                        | 274                                        | 930                                | 22                               | 13                                                    |

<sup>(1)</sup>N.D. = not determined

TABLE V

| Molar Ratio of Formaldehyde to Carbamate | Initial pH | Reaction Time (hrs.) | Reaction Temperature (°C.) | Dry Crease Recovery Warp+Filling (degrees) | Tear Strength Warp+Filling (grams) | Tensile Strength, Filling (lbs.) | Loss in Tensile Strength Due to Retained Chlorine (%) |
|------------------------------------------|------------|----------------------|----------------------------|--------------------------------------------|------------------------------------|----------------------------------|-------------------------------------------------------|
| 1:1                                      | 10         | 2                    | 103                        | 197                                        | 1170                               | 27                               | N.D. <sup>(1)</sup>                                   |
| 1.5:1                                    | 10         | 2                    | 103                        | 231                                        | 1120                               | 24                               | N.D.                                                  |
| 2:1                                      | 10         | 2                    | 103                        | 267                                        | 1040                               | 23                               | 7                                                     |
| 2.5:1                                    | 10         | 2                    | 103                        | 273                                        | 960                                | 22                               | 5                                                     |
| 3:1                                      | 10         | 2                    | 103                        | 283                                        | 930                                | 19                               | 4                                                     |

<sup>(1)</sup>N.D. = not determined

TABLE VI

| Molar Ratio of Formaldehyde to Carbamate | Initial pH | Reaction Time (hrs.) | Reaction Temperature (°C.) | Dry Crease Recovery Warp+Filling (degrees) | Tear Strength Warp+Filling (grams) | Tensile Strength, Filling (lbs.) | Loss in Tensile Strength Due to Retained Chlorine (%) |
|------------------------------------------|------------|----------------------|----------------------------|--------------------------------------------|------------------------------------|----------------------------------|-------------------------------------------------------|
| 2.2:1                                    | 10         | 2                    | 103                        | 258                                        | 1090                               | 26                               | 12                                                    |
| 2.2:1                                    | 8          | 2                    | 103                        | 254                                        | 1010                               | 23                               | 23                                                    |
| 2.2:1                                    | 6          | 2                    | 103                        | 264                                        | 1020                               | 24                               | 10                                                    |
| 2.2:1                                    | 4          | 2                    | 103                        | 257                                        | 1070                               | 25                               | 21                                                    |
| 2.2:1                                    | 10         | 0.25                 | 103                        | 265                                        | 1040                               | 26                               | 10                                                    |
| 2.2:1                                    | 10         | 0.5                  | 103                        | 263                                        | 1040                               | 24                               | 5                                                     |
| 2.2:1                                    | 10         | 1                    | 103                        | 259                                        | 1060                               | 27                               | 4                                                     |
| 2.2:1                                    | 10         | 5                    | 103                        | 260                                        | 1120                               | 22                               | 12                                                    |
| 2.2:1                                    | 10         | 2                    | 55                         | 253                                        | 1020                               | 20                               | 23                                                    |
| 2.2:1                                    | 10         | 2                    | 85                         | 257                                        | 1070                               | 28                               | 25                                                    |

methoxyethyl carbamates as a finishing agent for cellulosic textile fabrics. In the first test series, the fabric employed was a cotton printcloth having a thread count of 80 × 80, a dry crease recovery of 158°, a tear strength (warp + filling) of 1,180 grams, and a tensile strength (filling) of 37 lbs; the catalyst was MgCl<sub>2</sub>·6H<sub>2</sub>O; the add-on was 4% of methylated methoxyethyl carbamate and 1.2% of catalyst; and the treated fabric was dried for 1.5 minutes at 150°C. and cured for 1.25 minutes at 175°C. In the second test series, the same cotton printcloth was employed; the catalyst was Zn(NO<sub>3</sub>)<sub>2</sub>·6H<sub>2</sub>O; the add-on was 4% of methylated methoxyethyl carbamate and 0.2% of catalyst; and the treated fabric was dried for 1.5 minutes at 150°C. and cured for 1.25 minutes at 165°C. In the third test series, the fabric was a cotton broadcloth having a thread count of 136 × 64, a dry crease recovery of 155°, a tear strength (warp + filling) of 1,520 grams, and a tensile strength (filling) of 61 lbs; the catalyst was MgCl<sub>2</sub>·6H<sub>2</sub>O; the add-on was 4% of methylated methoxyethyl carbamate and 1.6% of catalyst; and the treated fabric was dried for 1.5 minutes at 150°C. and cured for 1.25 minutes at 175°C. The reaction condi-

50  
60  
65  
70  
75  
80  
85  
90  
95  
100

As evidenced by the data in Tables IV, V and VI, the methylolated alkoxyalkyl carbamate finishing agents of the present invention can be prepared over a relatively broad range of methylolation conditions and still perform effectively. The molar ratio of formaldehyde to alkoxyalkyl carbamate is the most significant variable, with crease recovery increasing and both tear strength and tensile strength decreasing with increasing formaldehyde to alkoxyalkyl carbamate ratios.

### EXAMPLE 4

Methylolated methoxyethyl carbamate and methylolated hydroxyethyl carbamate were evaluated as finishing agents for cotton fabric using various methylolation conditions and under varied fabric treating and curing conditions. The methylolation and fabric treating conditions are summarized for convenience in Table VII below, while the properties of the treated fabric are summarized in Table VIII. In each instance, the catalyst employed was MgCl<sub>2</sub>·6H<sub>2</sub>O and the treating bath contained 0.1 per cent TERGITOL TMN. The fabric employed was a desized, scoured, bleached and mercerized white cotton printcloth having a thread count of

80 × 80 and in each instance it was padded with a Butterworth Laboratory Padder at a wet pick-up of 80% and then dried on a pin tenter frame at 150°C. for 1.5 minutes.

Although the invention has been illustrated by the preceding examples, it is not to be construed as limited to the materials employed therein, but rather the invention encompasses the generic area as hereinbefore dis-

TABLE VII

| Test No. | Finishing Agent                    | Methylation Conditions                   |                      |             |             | Treating Bath pH | Fabric Treatment            |                 | Curing Temperature (°F.) | Curing Time (mins.) |
|----------|------------------------------------|------------------------------------------|----------------------|-------------|-------------|------------------|-----------------------------|-----------------|--------------------------|---------------------|
|          |                                    | Molar Ratio of Formaldehyde to Carbamate | pH                   | Time (Hrs.) | Temp. (°C.) |                  | Add-On (% on wt. of fabric) | Finishing Agent | Catalyst                 |                     |
| A-1      | Methyloated methoxyethyl carbamate | 2.2 <sup>(1)</sup>                       | 10 <sup>(3)</sup>    | 2           | Reflux      | 7.0              | 4                           | 1.6             | 350                      | 1.25                |
| A-2      | do.                                | 2.2 <sup>(1)</sup>                       | 10 <sup>(3)</sup>    | 2           | Reflux      | 4.5              | 4                           | 1.6             | 320                      | 3.0                 |
| A-3      | do.                                | 2.2 <sup>(1)</sup>                       | 10 <sup>(3)</sup>    | 2           | Reflux      | 4.5              | 4                           | 1.6             | 350                      | 1.25                |
| B-1      | Methyloated hydroxyethyl carbamate | 3.3 <sup>(1)</sup>                       | 10 <sup>(3)</sup>    | 2           | Reflux      | 7.0              | 4                           | 1.6             | 350                      | 1.25                |
| B-2      | do.                                | 2.5 <sup>(2)</sup>                       | 10-11 <sup>(4)</sup> | 2           | 50          | 4.5              | 4                           | 1.6             | 320                      | 3.0                 |
| B-3      | do.                                | 2.5 <sup>(2)</sup>                       | 10-11 <sup>(4)</sup> | 2           | 50          | 4.5              | 4                           | 1.6             | 350                      | 1.25                |
| B-4      | do.                                | 2.2 <sup>(1)</sup>                       | 10 <sup>(3)</sup>    | 2           | Reflux      | 7.0              | 4                           | 1.6             | 350                      | 1.25                |
| B-5      | do.                                | 2.2 <sup>(1)</sup>                       | 10.5 <sup>(4)</sup>  | 2           | 50          | 7.0              | 4                           | 1.6             | 350                      | 1.25                |
| B-6      | do.                                | 2.2 <sup>(1)</sup>                       | 10.5 <sup>(4)</sup>  | 2           | 50          | 4.5              | 4                           | 1.6             | 350                      | 1.25                |
| B-7      | do.                                | 2.5 <sup>(2)</sup>                       | 10-11 <sup>(4)</sup> | 2           | 50          | 7.0              | 4                           | 1.6             | 350                      | 1.25                |

<sup>(1)</sup>Methylation with p-formaldehyde (95%)

<sup>(2)</sup>Methylation with formalin (37.5%)

<sup>(3)</sup>Initial pH

<sup>(4)</sup>Constant pH throughout methylation reaction

TABLE VIII

| Test No. | Finishing Agent                    | Dry Crease Recovery Warp+Filling (degrees) | Tear Strength Warp/Filling (grams) | Tensile Strength Filling (lbs.) | Wash-Wear Rating    |          | Loss in Tensile Strength Due to Retained Chlorine (%) |
|----------|------------------------------------|--------------------------------------------|------------------------------------|---------------------------------|---------------------|----------|-------------------------------------------------------|
|          |                                    |                                            |                                    |                                 | Tumble Dry          | Spin Dry |                                                       |
| A-1      | Methyloated methoxyethyl carbamate | 255                                        | 450/210                            | 23                              | 4                   | 3-       | 2                                                     |
| A-2      | do.                                | 263                                        | 460/200                            | 20                              | N.D. <sup>(1)</sup> | N.D.     | 3                                                     |
| A-3      | do.                                | 260                                        | 460/170                            | 19                              | 4+                  | 3+       | 6                                                     |
| B-1      | Methyloated hydroxyethyl carbamate | 257                                        | 500/210                            | 23                              | 4+                  | 3        | 0                                                     |
| B-2      | do.                                | 253                                        | 460/200                            | 23                              | N.D.                | N.D.     | 26                                                    |
| B-3      | do.                                | 260                                        | 530/220                            | 23                              | N.D.                | N.D.     | 45                                                    |
| B-4      | do.                                | 244                                        | 500/220                            | 23                              | 4                   | 3+       | 60                                                    |
| B-5      | do.                                | 245                                        | 530/210                            | 23                              | 4                   | 3-       | 87                                                    |
| B-6      | do.                                | 239                                        | 530/220                            | 23                              | 4                   | 3+       | 87                                                    |
| B-7      | do.                                | 243                                        | 530/260                            | 20                              | N.D.                | N.D.     | 87                                                    |

<sup>(1)</sup>N.D. = not determined

As evidenced by the data in Tables VII and VIII, methyloated hydroxyethyl carbamate will provide good resistance to chlorine damage only if a very high formaldehyde to carbamate ratio is employed in effecting the methylation, with the resulting disadvantage of a very strong formaldehyde odor in the fabric. Moreover, changes in the pH of the treating bath or the curing conditions strongly influence the resistance to chlorine damage for fabric treated with methyloated hydroxyethyl carbamate, but have little effect on the resistance to chlorine damage of fabric treated with methyloated methoxyethyl carbamate. Accordingly, much less stringent control of fabric treating conditions is permissible with the methyloated methoxyethyl carbamate. This is an important distinction between the methyloated alkoxyalkyl carbamate finishing agents of this invention and the methyloated hydroxyalkyl carbamate finishing agents of the prior art.

closed. Various changes and modifications can be made in practicing the present invention without departing from it and therefore it is intended to include in the scope of the appended claims all such modifications and variations as may be apparent to those skilled in the art from the description and illustrative examples given herein.

What is claimed is:

1. A process for treating cellulosic textile fabric comprising the step of applying to said textile fabric at elevated temperatures in the presence of an acid catalyst an effective amount of the product of the reaction of formaldehyde with an alkoxyalkyl carbamate of the general formula:

65

0

"



wherein R is an alkyl group of 1 to 8 carbon atoms, R' is an alkylene radical of 2 carbon atoms, and n is an integer having a value of 1, said reaction being conducted at from about 20°C. to about the reflux temperature of the reaction mixture for a period of time from about 10 minutes to about 24 hours at an initial pH of from about four to about ten in a ratio of about 1.5 to about three moles of formaldehyde per mole of alkoxyalkyl carbamate.

2. The process of claim 1 wherein R is an alkyl group of 1 to 4 carbon atoms.

3. In a method for imparting wash-wear properties to cellulosic fabrics by treatment with a cross-linking agent followed by curing at an elevated temperature, the improvement for obtaining improved chlorine resistance which comprises employing as the cross-linking agent a product obtained by the reaction of formaldehyde in an aqueous alkaline solution with a glycol ether carbamate having the formula:

5



wherein R is ethyl; R' is hydrogen; and X is 1.

4. In a method for imparting wash-wear properties to cellulosic fabrics by treatment with a cross-linking agent followed by curing at an elevated temperature, the improvement for obtaining improved chlorine resistance which comprises employing as the cross-linking agent a product obtained by the reaction of formaldehyde in an aqueous alkaline solution with a glycol ether carbamate having the formula:

15



20 wherein R is methyl; R' is hydrogen; and x is 1.

\* \* \* \* \*

25

30

35

40

45

50

55

60

65

UNITED STATES PATENT OFFICE  
CERTIFICATE OF CORRECTION

Patent No. 3,871,822 Dated March 18, 1975

Inventor(s) H. G. Goodman, Jr. et al

It is certified that error appears in the above-identified patent and that said Letters Patent are hereby corrected as shown below:

Column 1, lines 24-25 should read:

"such as hydroxyethyl or hydroxypropyl carbamate, and have been observed to suffer from certain deficiencies, for example, with re-".

Column 6, line 9, "was" should read --wax--.

Column 10, line 4, the word "reaction" should appear after "differing".

Signed and Sealed this  
ninth Day of September 1975

[SEAL]

Attest:

**RUTH C. MASON**  
*Attesting Officer*

**C. MARSHALL DANN**  
*Commissioner of Patents and Trademarks*

### **Disclaimer**

3,871,822.—*Henry G. Goodman, Jr.*, White Plains, *Carol A. Dupraz*, Flushing (Corona), and *George H. Lourigan*, New City, N.Y. TREATMENT OF CELLULOSIC TEXTILE FABRICS WITH METHYLOLATED ALKOXYALKYL CARBAMATES. Patent dated Mar. 18, 1975. Disclaimer filed July 8, 1975, by the assignee, *Union Carbide Corporation*.

Hereby enters this disclaimer to claims 1 to 4 of said patent.

[*Official Gazette February 10, 1976.*]